

May 19, 1953

M. B. VORDAHL ET AL

2,639,244

METAL FINISHING METHOD

Filed July 15, 1950

2 Sheets-Sheet 1



Fig. 1

INVENTORS  
MILTON B. VORDAHL  
ROBERT H. GRACE  
PAUL H. ECCLESTON  
BY  
a. *Greene J. H.*  
*John H. Lewis Jr.*  
ATTORNEYS

May 19, 1953

M. B. VORDAHL ET AL  
METAL FINISHING METHOD

2,639,244

Filed July 15, 1950

2 Sheets-Sheet 2



## UNITED STATES PATENT OFFICE

2,639,244

## METAL FINISHING METHOD

Milton B. Vordahl, Trumbull, Conn., Robert H. Grace, Athol, Mass., and Paul H. Eccleston, Ilion, N. Y., assignors to Remington Arms Company, Inc., Bridgeport, Conn., a corporation of Delaware

Application July 15, 1950, Serial No. 174,062

10 Claims. (Cl. 148—6.11)

1

This application is a continuation-in-part of our prior applications of the same title, Serial Number 41,826, filed July 31, 1948, and Serial Number 113,342, filed August 31, 1949, both now abandoned. The additions and corrections made in this application are the result of further extensive production and laboratory experience with this method of finishing.

This invention relates to an improved finish for metallic articles and to a method of applying such a finish. The invention has been found to be particularly effective in black finishing articles formed of ferrous metal. The invention provides a useful finish for firearms and parts thereof, wire, strip, chain and other articles.

The objects of this invention are the provision of an attractive, durable, and corrosion resistant finish for metallic articles which may be conveniently and economically applied on a production basis.

An additional object is the development of a process which will produce uniform attractive coatings upon iron or steel, including the so-called "stainless steels" and which may be applied, with equally good results, to nickel, cobalt, and manganese, or to alloys including 50% or more by weight of one or more of the metals in the group consisting of iron, cobalt, nickel, and manganese.

Heretofore, the firearms finish which most nearly met the requirements of the industry has been that applied by the time-honored method of browning. This process may be briefly outlined as one in which a polished, thoroughly clean item is subjected to the following treatment:

1. Plug or rustproof interior surfaces.
2. Coat exterior with a rustproducing acid.
3. Allow rusting to proceed in a high humidity atmosphere.
4. Boil to convert the red oxide to a black oxide.
5. Wire brush or otherwise remove any non-adherent oxide.
6. Repeat each of steps 2, 3, 4, and 5 at least once and for as many as 5 or 6 cycles with very high grade arms.
7. Dye the relatively porous oxide coating and oil.

The quality of the finish is dependent upon the degree of initial polish and cleanliness of the workpiece. The depth of color and the durability of the finish are largely dependent upon the number of cycles of rusting, conversion and carding, which is the name applied by the arms industry to the step of wire brushing to remove non-adherent oxides. This process is time con-

2

suming and requires an excessive amount of hand work. Since it is a rusting process, it is almost wholly ineffective when attempts are made to apply it to rustless or stainless steels.

There are a number of fast processes for producing blue or black finishes on firearms but in one way or another such processes are inadequate for high quality work. For example, the phosphate coatings widely used on military firearms have a dead grey or dull black appearance. The so-called "oxide black" processes which involve boiling the parts in water solutions, including various caustics and/or nitrates or nitrites of the alkali metals, produce reasonably attractive finishes which have but little durability or corrosion resistance.

This invention resides in the discovery that polished, thoroughly clean articles, such as firearms, wire, or continuous strip, may be treated at relatively low temperatures in a molten bath of one or more alkali metal cyanides by a process which except for the low temperature is analogous to the well-known cyanide hardening processes followed, after suitable cleaning, by treatment in a relatively low temperature molten salt bath composed principally of an alkali metal nitrate and which may include also the hydroxide of an alkali metal. This process produces an exceptionally attractive, durable, and corrosion resistant finish which may be applied to all surfaces of the material. The process is particularly economical since it does not require the handling of individual pieces but permits small parts to be loaded in suitable racks holding several hundred items and moved by suitable conveyors through the successive steps. The nature of the process also permits continuous operation with materials in the form of wire, strip, or chain.

We have found that the process is effective when applied to iron, nickel, cobalt and manganese and to alloys in which 50% or more by weight is of one or more of the metals selected from the above group. In any alloy of this group the presence of small amounts of copper appears to improve the depth and richness of the color which in all cases is substantially black. It may be noted, however, that pure nickel and some of the high nickel alloys show a slightly brownish cast and that variations in processing, particularly relative to the temperature of the nitrate bath permit variations in density of the color ranging, for example, with carbon steel, from a semi-transparent blue black to a very dense black.

The process cannot be applied to pure molybde-

rium, tungsten, or chromium, all of which dissolve in the nitrate bath, and alloys including 50% or more of such metals have been noted as being subject to etching and other surface attack in the nitrate bath. The process is ineffective with the noble metals, and obviously should not be applied to any metal or alloy which cannot be exposed to temperatures between 940° F. and 1050° F. This obviously limits its application to steels which will not have the temper drawn an undesirable amount at those temperatures.

The exact nature of the invention, as well as other objects and advantages thereof, will more clearly appear from consideration of the following specification, referring to the drawing, in which:

Fig. 1 is a flow sheet outlining the preferred batch process of handling relatively small parts such as gun components.

Fig. 2 is a graph on which melting point and cost have been plotted for various percentages of sodium and potassium cyanide.

The specific description following will, in one section, discuss the invention in its application to firearms and parts thereof as a batch process. In another section a continuous process will be briefly described. It must, however, be recognized that the process and finish secured thereby are essentially the same regardless of the specific article or the use to which it may be put.

#### Batch process

The nature of the batch process is such that large quantities of parts may be handled simultaneously. Thus, for most efficient operation, it is contemplated that suitable fixtures or racks may be employed and transported from step to step by means of a monorail and hoist travelling thereon. Suitable racks hold, for example, 225 firearm barrels or 640 firearm receivers. The design of such racks is not particularly critical, but the following general points should be observed. For uniform coloring, the racks should support the work with the minimum of surface contact to enable the active agents to reach all surfaces. Each rack should include a shield to deflect back into the furnace any material expelled as a result of placing a load of hot work therein. For greatest economy in the operation of the process, the racks should present a minimum of surface area and no re-entrant pockets which might trap salt and add materially to the inevitable "drag-out" from the baths. In repeated use of the racks there is a tendency for the cyanide to creep into pin holes in welded areas which causes small but violent explosions when the rack is placed in the nitrate bath, thereby causing deterioration of welded joints. It is therefore preferable to design the racks to avoid any welds below the line of maximum immersion in the salts.

#### Clean

Unlike the browning process, our process does not mask surface irregularities by filling in depressions. Accordingly, the metal surface should be prepared initially by grinding, polishing, blasting or other means to secure the desired surface finish and to remove any scale or rolling "skin."

After the parts have been loaded into the racks the first step is a cleaning or degreasing operation. Satisfactory results have been obtained by the use of alkaline type cleaners such as water solutions of 3 to 6 ounces per gallon of sodium metasilicate with about 5% of a suitable wetting agent such as alkyl lauryl sulfonate or by water solutions of proprietary alkaline cleaners under-

stood to contain caustics, sodium pyro or metasilicate, sodium carbonate, a wetting agent, and possibly other ingredients.

Such cleaning solutions may be used in a tank deep enough to cover the load of work by at least three inches and may be maintained at a temperature at or near boiling. A range of 208° to 212° F. has been satisfactory. Mechanical agitation of the solution is preferable to insure thorough cleaning and it is desirable to move the rack completely in and out of solution several times at intervals during the cleaning treatment. A period of from ten to thirty minutes, depending on the type and amount of dirt, oil, etc., to be removed, is generally sufficient to insure thorough cleaning. Particular attention should be paid to relatively inaccessible surfaces such as the bore of a barrel and if difficulty is found in achieving thorough cleaning, it may be necessary to wipe out the bore with a suitable cleaner as a preliminary to placing the work in the racks. Excessive time in alkaline cleaning bath beyond that necessary for thorough cleaning should, however, be avoided as in several instances poor work has been traced back to this cause.

The use of vapor degreasing solutions such as trichlorethylene has also been found to be satisfactory. When this type of cleaning is used, it is practical to eliminate the subsequent two rinses and the drying operation and go directly from "Clean" to "Cyanide." It is essential that the work be clean before coloring is commenced if satisfactory results are to be obtained.

#### Rinse

Upon removal from the cleaner, the rack load of parts is immersed in a cold water rinse tank to remove any adhering cleaner and to serve as a check on cleanliness. It will be generally satisfactory to examine the work for water breaks at this point, and if none are found, it may be assumed that the preceding cleaning step has accomplished its purpose. Otherwise, the cleaning treatment should be repeated. To remove adherent cleaner, it is advisable to move the work up and down several times. There should be continual circulation from an inlet at the bottom of the tank and overflow at the top, and it is helpful to materially increase the flow for one or more minutes during immersion to assist in sweeping the surface of the tank free of floating cleaner so that as the work is removed it will not be recoated with cleaning compound.

#### Hot rinse

The cold water rinse may be followed by a hot water rinse in a similar tank provided with steam heating coils. For example, in one installation such a tank is permitted to idle at a temperature of around 150° F. and normally overflows enough to keep the water clean. When the rack of work is placed therein the inflow of water is stopped and the temperature permitted to rise to or near the boiling point. A range of 208° to 212° F. has been found satisfactory and a time of immersion of 5 minutes is adequate.

Since the work is now chemically clean, any but the stainless materials will be quite susceptible to rusting and should not be exposed to air until the 5 minute immersion period is over, whereupon the work should be removed and transferred to the drier as quickly as possible.

#### Dry

The step of drying after rinsing is essential to avoid the explosion hazard of transferring water

into the molten cyanide bath; although, as previously noted, it may be omitted if vapor degreasing equipment is used. The drier is essentially a gas or otherwise heated cabinet, which may be maintained at a temperature of approximately 300° F. and provided with a blower to insure a rapid circulation of air. As noted above, speed is desirable at this stage of the process and the work should be placed in the drier and dried as quickly as possible. The heat of the work as it comes from the hot rinse aids in drying.

#### Cyanide

After drying, the work may be removed from the drier and carefully inspected for water, rust, streaks, dirt or other undesirable material. If none of these are present, the work may be transferred to the pot of the cyanide furnace. After slowly lowering the work into the molten cyanide it should be moved up and down until there is no longer any encrustation of frozen cyanide thereon. This allows uniform operation from one load to the next, despite changes in load size. The work may then be allowed to remain immersed for 10 to 45 minutes at a temperature of not less than 940° F. The time is dependent upon a number of factors including process economics, the quality of the work output, and the cyanate content of the bath. In regard to process economics, it may be noted that 3 to 5 minutes in cyanide is usually adequate to prepare even stainless steel for receiving the black color. If color alone is the criteria, such short treatment is adequate and it would be unnecessary to use the more costly longer treatments. As to quality, it may be noted that the superlative wear and corrosion resistance achieved by this process will not usually be attained without at least 10 to 15 minutes in the cyanide bath. After about 45 minutes in cyanide the carbon steels and other less resistant materials are apt to be etched somewhat and longer times do not appear beneficial to either appearance, wear, or corrosion resistance of the coating. For the same quality of work the time in cyanide appears to vary in a roughly inverse ratio to the cyanate content of the bath. Thus, in the range of 15% to 20% cyanate about 15 minutes will produce a product equivalent to that produced in 5% cyanate after about 30 minutes.

For loads of work involving a considerable weight of material, it is desirable to preheat the furnace above 940° F. by about 2° F. for each 10 pounds of work before immersing the work, to provide a thermal head and to thereby avoid reducing the temperature materially below 940° F. as a result of heat transfer to the work. Alternate methods of achieving the same end are the use of oversized furnaces or the provision of heating devices capable of providing a temporarily stepped-up heat input comparable to the heat transfer to the work.

A suitable furnace must be capable of immersing the largest load of work to be processed and should provide some room for expansion of the cyanide salts. A preferred composition for the bath is the low melting eutectic mixture of sodium cyanide and potassium cyanide in proportions respectively of 60 and 40 parts by weight. However, the alkali metal cyanide is the active material and other proportions or a single salt may be used with good results if the variations in melting point are suitably observed. Fig. 2 is a graph in which the proportions of sodium and potassium cyanide are plotted against melt-

ing point and price of the mixed salts. It will be noted that the cheaper sodium cyanide has a much higher melting point than the eutectic mixture and therefore the cost of heating the bath and the likelihood of drawing the temper of heat-treated parts is increased. As noted, we prefer the eutectic mixture but, under conditions where heating costs are lower and heat damage not a factor, sodium cyanide may be preferable. For heat treated parts such as most firearm components, a temperature of 1050° F. is about the maximum which can be tolerated without drawing the temper to an undesirable extent. It may be noted that use of the bath results in increasing cyanate content and reduces the melting point below that indicated on the curve which is based on the fresh salts.

To compensate for drag-out and to obtain uniform activity of the bath, we have found that it is desirable to add 60% sodium cyanide and 40% potassium cyanide salts to the bath on a daily basis. It should also be noted that maximum wear and corrosion resistance is not attained until a fresh bath has been aged at working temperature for approximately two weeks. This aging appears to have the function of building up the cyanate content (CNO) of the bath to a degree of 5% or higher. After this degree of cyanate content has been reached, efforts should be directed at minimizing the oxidation responsible for cyanate build-up to avoid etching of work, racks and furnace pot. It appears to be desirable to hold the cyanate content below 20% or the work may be etched to a degree which cannot be tolerated. A tightly fitting cover for the cyanide bath is of assistance in reducing cyanate build-up and is necessary to prevent water and other materials splashing into the cyanide bath and to cut down on heat loss. Floating covers which prevent the access of air to the surface of the cyanide have also proven useful.

As the bath is used, certain materials therefrom form an encrustation on the sidewalls of the pot above the fluid salt level and also on the floating covers if these are used. Chemical analysis shows this material to be predominantly sodium carbonate, with some cyanide, and cyanate of sodium and the iron content has been found to be as high as 0.28%. Indications are that if this material is permitted to return to the molten bath trouble will be experienced in subsequent coloring. Accordingly, each morning this encrustation is collected with a suitable skimming and scraping implement, and discarded.

Another control technique which appears to be effective is a weekly sludging of the cyanide bath at a somewhat reduced temperature. Accordingly, each week-end the temperature may be reduced as far as possible without loss of fluidity in the bath, and before starting up again the sludge which has settled to the bottom of the bath is dipped out with suitably shaped dippers. In this way, 25 to 50 pounds of sludge may be removed per week.

This low temperature cyaniding produces with each of the materials to which the process may be applied a thin case hardened surface not usually over about .0001 inch thick and, in addition, has some effect not fully understood which increases by several times the wear and corrosion resistance of the black finish subsequently applied thereto. Stainless steel and certain other materials such as "Stellite" and

"Hastelloy" of various grades cannot be colored in a nitrate bath without this preliminary step.

#### Cyanide wash

Upon completion of the time cycle in the cyanide bath, the work should be raised and lowered several times, allowed to drain briefly, and moved to the wash tank. When heated rifle barrels or other tubular members are lowered vertically into a water bath, an effect analogous to the action of the well-known percolator causes a jet of water to spurt therefrom. To guard against this, a cover is placed upon each rack before washing unless the rack design is such as to inherently provide for deflecting this water back to the wash tank. Unless the cyanide furnace is remote from the wash tank, suitable precautions should be taken to prevent splashing water thereinto.

It should be noted that it is quite difficult to remove adhering cyanide if it has once been allowed to cool and dry on the work. Accordingly, an immediate and thorough washing is desirable. Hot or boiling water has been generally satisfactory as a washing agent, but about 3% sodium hydroxide or a small percentage of one of the alkaline cleaners added to the wash water is beneficial. The main objective is to get the surface as near chemically clean as possible.

It has been found to be undesirable to wash in cold water as the thermal shock tends to cause warpage of barrels and other precision parts, and, of course, the removal of adhering salts is more difficult. A desirable minimum temperature for the wash water has been found to be 180° F.

The cyanide wash tank is an installation which may be cited as an example is normally maintained in an over-flowing condition at a minimum of 180° F. When the work has been fully immersed, the temperature is allowed to rise to boiling, largely by heat transfer from the work, to assist in removing adhering salts. After turbulence has ceased, the work may be removed for transfer to the succeeding hot rinse.

#### Hot rinse

A further rinsing is sometimes desirable after the cyanide wash, and this rinse should also be in hot water. For example, this step may be carried out in a tank maintained between about 208° and 212° F., and slowly overflowing. The rack of work may be placed therein for a period of from 3 to 5 minutes, being moved up and down several times at the beginning and end of the cycle.

#### Work transfer

As noted previously, it is desirable to avoid the use of racks with welded joints beneath the salt line. If it has not been possible to do this, it may be found that repeated use will have caused deterioration of the welded joints resulting in small cracks or pits which may entrap cyanide salts and retain them through the washing step. If welded racks having such joints are used, it is preferable to transfer the work after rinsing to a rack which is used only in the subsequent steps. Otherwise, local explosions of some violence may result when the racks containing entrapped cyanide are placed in the nitre bath to follow. If this transfer is made, clean gloves should be worn to prevent contamination of the work.

#### Dry

Whether or not the work is transferred to an-

other rack, it is thoroughly dried, and this operation may be performed conveniently in a drying cabinet substantially the same as that used after cleaning. For fast drying the cabinet may, for example, be maintained at substantially 300° F. for substantially 20 minutes and provided with a blower to produce a current of heated air.

#### Nitre

The nitre bath is a molten salt bath in which the active ingredient is a nitrate of an alkali metal with which a caustic alkali or other derivatives may be used. We prefer to use a nitre bath which consists initially of 90 parts by weight of sodium nitrate and 10 parts of sodium hydroxide. It is this bath which imparts the black color to the work, and experience has shown that the shade of the color is to a considerable extent dependent on temperature. For example, 900° F. yields a reddish black product, 950° F. a blue black, and 1000° F. a dark black. The color is not satisfactory for firearm components if the temperature is allowed to drop during coloring below 940° F. It is therefore desirable to preheat the bath or in some other way provide a thermal head sufficient to offset heat transfer to the work. For example, with a furnace holding between 1600 and 2000 pounds of molten salt, it has been found sufficient to preheat the bath before receiving the work by about 2° F., for each 10 pounds of work to be placed therein. Thus, with a load of 150 barrels, weighing about 445 pounds, it is desirable that the nitre bath cited as an example be preheated to about 1040° F., or a raise of 100° F. By so controlling the thermal head, it is possible, and desirable, to insure that the work, during most of the time it is immersed in the bath, will be maintained at a temperature within the range of about 940° F. to 1050° F.

As in the case of the cyanide bath, a maximum temperature of 1050° F. should be observed for heat treated parts to prevent drawing the temper to an undesirable extent.

All work must be thoroughly dry before being placed in this furnace, and upon removal from the drier a careful inspection must be made to verify that this is so. The work may then be slowly lowered into the bath but the lowering should not be interrupted unless absolutely necessary until the parts have been completely covered, or a ring on the work may result. After complete immersion, the work may be moved in and out of the bath until the work seems to have taken on its deepest color, which will be after the work has come fully up to temperature. The work may then be allowed to remain in the bath for a total period of from not less than about 15 minutes and preferably 30 to 60 minutes, after which it may be raised and lowered several times. As the work is removed from the furnace pot, it may be inspected for color. If any areas of a hard red oxide are noted, the work should be returned to the furnace for another 20 minutes.

Although we have above noted our preference for a bath of 90% sodium nitrate and 10% sodium hydroxide, it may be noted that the caustic alkali may be omitted with only slight detriment to the color. It appears that the effect of the caustic is to produce a slight etching of the surface and to give the impression of a deeper richer black. The straight nitrate tends to produce a semi-transparent blue-black. The most generally attractive finish will be produced after the caustic content has been raised to about 5%;

and caustic contents higher than 15% etch the surface so severely as to destroy the polish and produce a semi-matte or dead appearing surface. It may also be noted that a sodium nitrate-manganese dioxide combination in a 50-to-1 ratio may be used with fair success, although the surface does not have an appearance as attractive as that produced by the nitrate-caustic combination.

As the bath is used, there appears to be a slow reaction between the bath and the carbon dioxide of the air which, among other things, produces sodium carbonate in the bath. After the carbonate content reaches about 20%, it appears to stabilize, and additional carbonate sludges out about as fast as it is formed, where it can be removed as it accumulates in the bottom of the furnace pot. In production operations, the exact relationship between carbonate content and caustic content has not been determined, but it has been noted that a failure to color properly to the desired deep color may usually be corrected by a slight increase in the caustic content.

As a routine control technique, daily additions to the bath of sodium nitrate and sodium hydroxide in a ratio of about 8 to 2 appear to be desirable in proportion to the amount of work processed. For example, in processing an average of 500 pounds of work per day, it was found that daily additions of 8 pounds of sodium nitrate and 2 pounds of sodium hydroxide were sufficient to keep the bath in proper working condition. As larger quantities of work are processed, it appears desirable to continue the addition of fresh salts in about the same proportion to the amount of work. These additions usually require that some of the old salt be bailed out and discarded as the loss of salt through drag-out seldom equals the amount of the daily additions.

#### Nitre wash

In the next step of the process, the work may be removed from the nitre furnace and washed to remove adhering salts and to lower the work toward room temperature. As in the case of the cyanide step, the salts from the nitre bath, particularly a reddish film, sometimes carried out, are quite difficult to remove if permitted to cool and dry on the work. For example, work which is air-cooled has an inferior color because of the reddish film which can then be removed only by abrasive polishing. 1 to 3 minutes exposure to the air during draining and transfer of the work does not appear to be critical, but materially longer delays should be avoided, if possible. Care should be taken to prevent splashing water into the hot nitre furnace and, as noted in connection with the cyanide wash, the racks should be covered to deflect the inevitable jet of water resulting from the contact of the hot work with the wash water. As in the case of the cyanide wash, severe thermal shocks should be avoided by the use of a hot wash water at a minimum of 180° F. having been found satisfactory.

The nitre wash may, for example, be in a continuously overflowing tank of water maintained at a minimum temperature of 180° F., toward which the work is slowly lowered until contact is made, after which the work may be lowered rapidly until completely immersed. The admission of water may then be increased and the tank allowed to overflow rapidly until the water runs clear. The work may remain in the water for about 5 minutes at a reduced rate of flow.

#### Hot oil

The final step in the process consists in immersing the work in a bath of hot oil which is to some extent absorbed in the coating and improves the appearance and corrosion resistance thereof. An oil-water emulsion consisting of a soluble oil and water in proportions of about two parts oil and four parts water has been found to be satisfactory. The incorporation of a durable wax is, in some cases desirable in order to reduce the tendency for the formation of an unattractive film of moisture upon handling with moist hands after the surface oil has been rubbed off. Such a lubricant is preferably applied hot—say at 120° F.—and the tank may be conveniently maintained at such temperature by means of a submerged steam coil. The work is preferably allowed to remain in this bath for at least 10 minutes. In use, an oil film appears to form on the surface of the bath and preferably, the bath should be agitated to disperse this film before raising the work.

After draining, the racks may be unloaded and the finished work forwarded for inspection and assembly.

#### Continuous process

There are many items, of which wire, continuous strip, particularly measuring tapes, and chain, particularly bicycle chain, are examples, which would benefit from the application of this process but which are not readily adaptable to batch operations. For such items, a continuous operation is desirable and may be readily provided by the use of suitable fixtures designed to hold a loop or loops of the material submerged in the treating pots. Obviously the rate of travel and length of the submerged loop may be adjusted to secure the desired time of immersion in each of the pots. Particularly with wire, many of the operating problems, such as the removal of adhering salts, are simplified.

Considering an illustrative arrangement for such continuous treatment, the material may be brought into the process at the cleaning bath in the box marked 2 on the drawing. If the material is considered to be divided into any convenient unit lengths, the feed may be arranged to draw the material through at a rate of travel of one unit of length in ten minutes and the guides may be arranged to hold three units of length submerged in the cleaning bath. Each increment of the material will therefore receive the recommended 30 minutes of submersion in the cleaner. 55 With wire and other simple forms 10 minutes or less seems adequate. The design of the fixtures guiding the material is not critical from any standpoint other than that of guiding without applying any undue frictional loadings. Particularly in the cleaner, and for smooth materials, the guides may take the form of wiping pads which assist in cleaning.

With bicycle chain and other more complicated forms the material should then be drawn through one or two rinse baths as used in the batch process, followed by passing through a heated drying chamber.

With wire and strip stock there is very little drawout from any of the baths and the washing and rinsing steps may sometimes be omitted and almost never need to be duplicated. After cleaning, a simple rinse by pulling the wire through a pad over and through which water is flowing is usually adequate. Drying is also quite simple and the most that is required is to pass the wire

through a heated chamber arranged to accommodate one or two unit lengths of wire at a time.

Ten minutes appears to be an adequate length of time for the cyanide treatment of wire and may be accomplished at the previously mentioned rate of travel by arranging the guides to hold one unit length of wire submerged at a time. Obviously 20 or 30 minutes will give a deeper cyanide case and is desirable with such material as bicycle chain. Such longer period may be provided for by arranging the guides to respectively hold two or three unit lengths of wire submerged at a time.

Wire has very little tendency to drag out cyanide salts and the wash following cyanide treatment need not be elaborate. Probably the minimum is to draw the wire through a pad in and through which water is being circulated and the maximum would be to draw the wire through a hot or boiling water bath in which one or two unit lengths could be submerged at a time. With such material as bicycle chain, however, several unit lengths should be submerged in substantially boiling water and a rinse should be performed in a second hot bath in order to ensure that the cyanide is completely removed. As before, the work may be dried by passing through a heated chamber.

Ten minutes in the nitre bath is usually adequate for wire and twenty to thirty should suffice for the heavier more complicated articles such as chain. As before, these times can be achieved at the previously discussed rate of travel by arranging the guides to hold one, two, or three units of length submerged in the bath at one time. The nitre wash may be carried out in the same manner as the previously described wash steps, preferably in hot water, and the work then passed through hot oil unless oil would exert an undesirable effect on the end product as in certain electrical applications of such treated wire.

With wire or other material of substantial strength, the entire process may be handled by a single winding and reeling unit at the discharge end which pulls the material from the delivery spool and through all of the process baths. With fine wire it is desirable to use several winding units at intervals between the baths to minimize the tensile strain on the wire.

This process has been particularly effective upon several variations of Nichrome used in fine wire form as resistance materials. In this application, in addition to color, the wire is materially improved in regard to tensile strength and its electrical properties and the dielectric effect of the coating are modified, in a way we do not understand but which seems to be of great interest to the producers of Nichrome resistance wire.

We do not intend to indicate that the continuous treatment of wire, strip, or other continuous articles for coloring or heat treatment is novel with us but simply wish to point out that our process, developed originally for batch application to small mechanical devices mounted in racks, can be successfully applied to the treatment of wire and like articles. Accordingly, we wish to note that we consider the appended claims to apply to a continuous as well as to a batch process.

#### *Effectiveness of the process*

By the batch process it has been possible to consistently produce on polished firearm parts a

5

10

20

25

30

35

40

45

50

55

60

65

70

deep blue-black color of superior appearance which is characterized by very high wear, scratch, and corrosion resistance. For example, comparative tests of identical arms parts subjected to the prior art treatments and to this process have been made on the basis of measuring the time necessary to produce equal degrees of corrosion on exposure to the conventional salt spray test. Several of these tests are tabulated below. The material is identical in each case and the treatment of the sample is indicated in the left hand column. The time indicated is that necessary in each case to produce an equivalent degree of corrosion on all samples in that column.

|                              | Test A  | Test B  | Test C |
|------------------------------|---------|---------|--------|
| Plain Steel                  | 10 min. | 30 min. | 1 hr.  |
| Plain Oxide Black            | 15 min. | 2½ hrs. | 2 hrs. |
| Cyanide Only                 | 20 min. | do      | do     |
| Conventional 4 Coat Browning | 10 min. | 14 hrs. | 5 hrs. |
| Cyanide+Nitre Black          | 83 min. |         |        |

Another comparative test which perhaps more accurately represents service conditions was performed with identical receivers for Model 512 Remington rifles. One set of samples was processed as disclosed herein and subsequently completely degreased to remove any of the oil which might have tended to mask the improvement in corrosion resistance due to the "Cyanide-Black" process. The other set of samples was processed by the conventional "Browning" technique and also degreased.

Both sets of samples were exposed in identical locations in the rusting room of the conventional "Browning" process which is accurately maintained at a constant 110° F. temperature and 70 percent relative humidity. After three weeks, samples of the browned receivers were removed and found to be badly rusted. Sample "Cyanide-Black" receivers were removed after 2½ years' exposure and showed no spots of rust or corrosion. At the present time "Cyanide-Black" receivers of this lot are still in the rusting room and, after more than three years' exposure, still show no rust spots. A recent sample of browned receivers, identical with those in the previous test and except for surface treatment identical with the "Cyanide-Black" receivers still in the rusting room, was removed after 3-weeks and 3-days' exposure and again the sample was badly rusted.

Further recent tests have also demonstrated the outstanding wear and corrosion resistance of the "Cyanide-Black" process. These tests were performed with a standard Taber abrasion and scratch tester. This machine provides a turntable upon which samples may be mounted and is arranged to be driven by suitable power. Over this turntable there is mounted an arm carrying a pair of rubber bonded abrasive wheels mounted so that the axis of the wheels is at an angle to the radius of the turntable. As the turntable rotates it is dragged under the wheel and, due to the angular position of the wheel axes, a component of the dragging force rotates the abrasive wheels at a relative slow rate. A revolution counter is provided to record the number of cycles to which each sample is subjected. The wheels are standardized and are resurfaced after each 500 cycles of rotation of the turntable. The loading on the arm may be selected to determine the severity of the test and the test is concluded when the surface finish has been abraded sufficiently to expose the underlying metal. In our

test we used identical samples of 18-8 stainless steel and SAE 1070 carbon steel. The carbon steel specimen and one stainless specimen were treated by the process here disclosed and the other stainless specimen was treated by the best available competitive method of blacking stainless steel.

In the comparative test, all test plates were thoroughly cleaned to remove all traces of oil and dirt. Standard Taber C-10 "Calibrase" wheels were used for abrading and a 500 gram load was applied to the wheels. After 1000 cycles the competitive process sample of stainless steel was clearly worn through, at 3000 cycles there was a clear break through with the "Cyanide-Black" carbon steel specimen, and at 5000 cycles the "Cyanide-Black" stainless sample showed only a questionable break through.

In the scratch test with this same equipment the arm is changed to utilize an arm holding a carbide cutter somewhat like a lathe threading tool and the specimen is moved thereunder by small increments of turntable movement. After each increment the loading on the arm is increased by 50 grams. The first break-through is readily apparent by visual inspection of the sample. The specimens were prepared as for the abrasion test and at a 450 gram loading the cutter penetrated the finish of the competitive process stainless specimen. The scratch test machine will not take more than 1000 grams load on the cutter and at that load neither the stainless nor carbon steel "Cyanide-Black" specimens showed any visible evidence of scratching.

Since in the most economical application of this process to firearms barrels the bore of the barrel is left open during processing, this same wear and corrosion resistant surface will be applied thereto. As a result, the bore is rendered highly resistant to mechanical abrasion and to corrosion from the chemical agents released by the burning of certain types of propellant powder and primers. As an example, a 12-gauge shotgun having its bore surface finished in this way has been fired with 5,000 rounds of ammunition of all available types, with no evidence that the coating has been affected in any way. Caliber .22 rifles have also been fired many thousands of rounds without evidence of mechanical wear or chemical corrosion of any surfaces.

The processes as presently practiced have been outlined in considerable detail. Obviously variations may be made therein without departing from the spirit of the invention and it should be clearly understood that it is intended to include within the scope of the appended claims all equivalent materials, proportions, and procedures. While extended experience with the process may indicate that not all of the control procedures outlined are necessary, their use appears to be advantageous for full scale production.

What is claimed is:

1. The process of securing a stable, uniform, substantially black coating upon an article having a surface of iron, nickel, cobalt, manganese, or of an alloy containing 50% or more by weight of one or more of said metals, said process comprising the steps of submerging the article in a first treating bath having as its essential ingredient a molten cyanide of at least one of the alkali metals at a temperature not less than about 940° F. for a period of time sufficient to develop a shallow hardened skin; and subsequently submerging the article in a second treating bath having as its essential ingredients a

molten nitrate of at least one of the alkali metals admixed with from 5% to 15% of alkali metal hydroxide, said second bath being maintained at a temperature not less than about 940° F. for a period of time sufficient to develop the black color, said first treating bath having been aged at substantially working temperatures and thereby partially oxidized to increase the cyanate content and thereafter controlled to maintain the cyanate content in a range between about five percent and about twenty percent.

2. The process as described in claim 1, said article being maintained in said first bath for a period of time not less than about ten minutes.

15 3. The process as described in claim 2, said article being maintained in said second bath for a period of time not less than about fifteen minutes.

4. The process as described in claim 3, said 20 first and second baths being maintained for substantially the entire period of immersion of said article in said baths in a temperature range between about 940° F. and about 1050° F.

5. The process as described in claim 4, said 25 article being immersed after removal from said first bath and again after removal from said second bath in heat absorbing, adherent salt dissolving, aqueous media maintained at a temperature not substantially less than about 180° F.

30 6. The process as described in claim 5, said first bath consisting initially of the product of the low melting eutectic mixture of sodium and potassium cyanides.

7. The process as described in claim 6, said 35 second bath consisting initially of the molten product of the admixture of substantially 90 percent sodium nitrate and substantially 10 percent sodium hydroxide.

8. The process of securing a stable, uniform, 40 substantially black coating upon an article having a surface of iron, nickel, cobalt, manganese, or of an alloy containing 50% or more by weight of one or more of said metals, said process comprising the steps of chemically cleaning all surfaces of said article; submerging said cleaned 45 article in a first treating bath having as essential ingredients a mixture of molten alkali metal cyanides maintained at a temperature between about 940° F. and about 1050° F. for a period of time between 10 and 45 minutes; freeing said article of adherent cyanide by immersing in water maintained at a temperature not less than about 180° F.; subsequently submerging said article in a second treating bath of a molten mixture including not less than about 65 percent molten alkali metal nitrate and not more than about 15 percent caustic alkali maintained at a temperature between about 940° F. and about 1050° F. for a period of time between about 15 and 60 minutes; freeing said article of adherent alkali metal salts by immersing in water maintained at a temperature not less than about 180° F.; and subsequently submerging said article in a heated, protective, oily material.

60 9. The process of securing a stable, uniform, substantially black coating upon a firearm component having a surface of iron, nickel, cobalt, manganese, or of an alloy containing 50% or more by weight of one or more of said metals, said process comprising the steps of chemically cleaning all surfaces of said component; submerging said cleaned component in a first treating bath having as essential ingredients a mixture of molten alkali metal cyanides maintained at a temperature between about 940° F. and about

70 75

150° F. for a period of time between 10 and 45 minutes; freeing said component of adherent cyanide by immersing in water maintained at a temperature not less than about 180° F.; subsequently submerging said component in a second treating bath of a molten mixture including not less than about 65 percent molten alkali metal nitrate and not more than about 15 percent caustic alkali maintained at a temperature between about 940° F. and about 1050° F. for a period of time between about 15 and 60 minutes; freeing said component of adherent alkali metal salts by immersing in water maintained at a temperature not less than about 180° F.; and subsequently submerging said component in a heated, 15 protective, oily material.

10. The process of securing a stable, uniform, substantially black coating upon the bore and exterior surface of a firearm barrel consisting of iron, nickel, cobalt, manganese, or of an alloy 20 containing 50% or more by weight of one or more of said metals, said process comprising the steps of chemically cleaning all surfaces of said barrel; submerging said cleaned article in a first treating bath having as essential ingredients a mixture of molten alkali metal cyanides maintained at a temperature between about 940° F. and about 150° F. for a period of time between 15 and 45 minutes; freeing said barrel of adherent cyanide by immersing in water maintained at a tem- 30

5  
10

perature not less than about 180° F.; subsequently submerging said article in a second treating bath of a molten mixture including not less than about 65 percent molten alkali metal nitrate and not more than about 15 percent caustic alkali maintained at a temperature between about 940° F. and about 1050° F. for a period of time between about 15 and 60 minutes; freeing said barrel of adherent alkali metal salts by immersing in water maintained at a temperature not less than about 180° F.; and subsequently submerging said barrel in a heated, protective, oily material.

MILTON B. VORDAHL.  
ROBERT H. GRACE.  
PAUL H. ECCLESTON.

References Cited in the file of this patent

UNITED STATES PATENTS

| Number    | Name      | Date          |
|-----------|-----------|---------------|
| 1,247,086 | Crowe     | Nov. 20, 1917 |
| 1,528,245 | Crapo     | Mar. 3, 1925  |
| 1,853,562 | Herr      | Apr. 12, 1932 |
| 1,988,217 | Sayles    | Jan. 15, 1935 |
| 2,370,959 | Holden    | Mar. 6, 1945  |
| 2,431,986 | Clingan   | Dec. 2, 1947  |
| 2,476,345 | Zavarella | July 19, 1949 |
| 2,513,302 | Field     | July 4, 1950  |